

# UNITED STATES PATENT OFFICE.

GEORGE E. FERGUSON, OF NEW YORK, N. Y., ASSIGNOR TO PYRENE MANUFACTURING COMPANY, A CORPORATION OF DELAWARE.

## FIRE-EXTINGUISHING AND FIREPROOFING COMPOSITION.

1,271,506.

Specification of Letters Patent.

Patented July 2, 1918.

No Drawing.

Application filed November 18, 1913. Serial No. 801,733.

To all whom it may concern:

Be it known that I, GEORGE E. FERGUSON, a citizen of the United States, and resident of the city, county, and State of New York, have invented certain new and useful Improvements in Fire-Extinguishing and Fireproofing Composition, of which the following is a specification.

This invention relates to a fire extinguishing composition and more particularly to a compound which will not only extinguish the flame but will also render the material fire-proof and thus prevent the re-ignition thereof from smoldering embers or other causes.

After a long series of experiments I have found that such a fire extinguishing and fire-proofing composition may be made up of a water solution of sodium silicate, borax, sodium ammonium phosphate and monosodium phosphate.

Sodium silicate or "water glass," (having a formula of  $Na_2Si_4O_9$ ) has been used in a number of different compounds for fire-proofing various materials. When "water-glass" is heated it gives a sandy pulverized mass, grayish white in color and extremely refractory when subjected to heat. If a coating of this material, when heated, could be caused to fuse into a skin or homogeneous covering, it would make an excellent fire-proofing material and with this end in view I added borax, a salt of sodium and boric acid, (having a formula of  $Na_2B_4O_7 \cdot 10H_2O$ ).

When borax is heated it gives off water and the remaining portion fuses to a colorless, transparent glass, commonly known as "borax glass"; the higher the heat the quicker and better it forms the glass. When borax is mixed with "water glass" and then heated the coating is excellent, being very tough and homogeneous, and forming an excellent fire-proof skin.

In extinguish wood fires, it has been found difficult heretofore to extinguish the burning embers. The large flame is easily extinguished, but the embers are the hardest to put out. Should a piece of wood having burning embers on it be placed in an atmosphere free from oxygen it would be instantly extinguished. Ammonia gas will make an oxygen free atmosphere, so if this gas could be generated and held about the

embers for an instant it would insure the complete extinguishing of any trace of fire.

With this end in view, sodium ammonium phosphate, commonly known as microcosmic salt, (having a formula of  $NaNH_4HPO_4$ ) was added to the mixture. Microcosmic salt when heated first melts and then decomposes, giving off ammonia gas and leaving a phosphate of soda. The ammonia gas is trapped for a short period of time under the skin produced by the heating of the sodium silicate and borax combination and instantly extinguishes the burning embers.

A part of the ammonia gas will also be mixed with the various gases emitted by the fire and will tend to combine with the acid portions of the fumes, thereby rendering them less obnoxious and corrosive. The phosphate of soda which remains of the decomposition products of the microcosmic salt forms one of the best fire-proofing materials obtainable.

Monosodium phosphate ( $NaH_2PO_4 \cdot H_2O$ ) is added to further increase the fire-proofing qualities of the liquid by enabling the percentage of phosphate to be increased, the "mono salt" being taken because of its greater solubility in water than the other phosphates of soda.

The portions which I have found advantageous are as follows:

100 c. c. of water glass, having specific gravity of 1.4289 at 15 deg. centigrade.

10 grams of borax, 10 grams of microcosmic salt and 4 grams of monosodium phosphate are then mixed in 100 c. c. of water. When the last three compounds are thoroughly dissolved the liquid which results is poured, with constant stirring, into the water glass.

It will thus be seen that this composition is capable of producing several useful results and that these results are accomplished in a novel manner by the co-action of the several ingredients of the composition when the same is used on a fire. A fire extinguishing gas is formed and held about the burning material by the fire-proof skin produced by the composition when subjected to the heat of the fire. This gas not only extinguishes the flame but also the smoldering embers, as already described, and also neutralizes the acid portions of the fumes from the fire. Finally, in addition to performing the above

noted functions, the fire-proof skin is left, forming a fire-proof coating which prevents re-ignition.

I do not wish to be understood as limiting my invention to the specific ingredients or to the exact proportions or method of making the composition herein set out as illustrative of a preferred embodiment of my invention, as it may be possible to substitute other ingredients or to vary the composition as defined in the appended claims without departing from the spirit of the invention.

What I claim is:—

1. A fire extinguishing composition composed of substances which, when exposed to the heat of the fire, give off ammonia gas and also produce a coating which holds said gas about the burning material.
2. A fire extinguishing composition composed of substances which, when subjected to the heat of the fire, give off ammonia gas and also deposit a fire-proofing coating on the burning material.
3. A fire extinguishing composition composed of substances which, when subjected to the heat of the fire, give off ammonia gas and also produce a fire-proof coating which first holds the ammonia gas about the burning material and is then deposited thereon as a coating.
4. A fire extinguishing composition composed of microcosmic salt in combination

with substances which when subjected to the heat of the fire produce a fire-proof coating about the burning material.

5. A fire-extinguishing and fire-proofing composition composed of sodium silicate, borax, and two different phosphates of sodium, one of said phosphates being adapted to evolve a fire-extinguishing gas.

6. A fire extinguishing and fire proofing composition composed of sodium silicate, borax, microcosmic salt and monosodium phosphate.

7. A fire - extinguishing and fire - proofing composition composed of borax and two different salts of sodium, one of said salts being adapted when acted upon by the heat of the fire to give off a fire-extinguishing gas and the other to deposit a fire proofing substance.

8. A fire - extinguishing and fire - proofing composition composed of substances which when subjected to the heat of the fire give off a fire-extinguishing gas and also deposit a fire-proofing coating on the burning material, and which when brought together will not react chemically in water solution.

Signed at the city, county and State of New York, this 13th day of November, 1913.

GEORGE E. FERGUSON.

Witnesses:

LEWIS J. DOOLITTLE,  
LUELLA F. LITTLE.